



US005912430A

# United States Patent [19]

Nielson

[11] Patent Number: 5,912,430

[45] Date of Patent: \*Jun. 15, 1999

[54] **PRESSABLE INFRARED ILLUMINANT COMPOSITIONS**[75] Inventor: **Daniel B. Nielson**, Brigham City, Utah[73] Assignee: **Cordant Technologies Inc.**, Brigham City, Utah

[\*] Notice: This patent is subject to a terminal disclaimer.

[21] Appl. No.: **08/386,327**[22] Filed: **Feb. 10, 1995**

## Related U.S. Application Data

[63] Continuation of application No. 07/913,841, Jul. 15, 1992, abandoned.

[51] **Int. Cl.<sup>6</sup>** ..... **C06B 45/10**[52] **U.S. Cl.** ..... **149/19.1**; 149/19.5; 149/19.6; 149/22; 149/61; 149/116; 102/336[58] **Field of Search** ..... 102/336; 149/19.1, 149/22, 61, 116, 19.5, 19.6[56] 

## References Cited

### U.S. PATENT DOCUMENTS

|           |         |                    |          |
|-----------|---------|--------------------|----------|
| 2,909,418 | 10/1959 | Pearsall           | 52/2     |
| 3,411,964 | 11/1968 | Douda              | 149/19   |
| 3,475,237 | 10/1969 | Lane et al.        | 149/22   |
| 3,617,403 | 11/1971 | Johnson            | 149/19   |
| 3,673,013 | 6/1972  | Lane et al.        | 149/116  |
| 3,677,842 | 7/1972  | Doris              | 149/19.1 |
| 3,706,611 | 12/1972 | Hastings           | 149/44   |
| 3,733,223 | 5/1973  | Lohkamp            | 149/116  |
| 3,888,177 | 6/1975  | Tyroler            | 149/116  |
| 3,895,578 | 7/1975  | Shaw et al.        | 102/336  |
| 3,951,705 | 4/1976  | Manicinelli et al. | 149/41   |
| 3,986,907 | 10/1976 | Dillehey           | 149/19.1 |

|           |         |              |         |
|-----------|---------|--------------|---------|
| 4,078,954 | 3/1978  | Bernardy     | 149/116 |
| 4,204,895 | 5/1980  | Webster      | 149/22  |
| 4,719,857 | 1/1988  | Spring       | 102/335 |
| 5,056,435 | 10/1991 | Jones et al. | 102/336 |
| 5,317,163 | 5/1994  | Obkircher    | 102/334 |

### FOREIGN PATENT DOCUMENTS

|           |         |                |   |
|-----------|---------|----------------|---|
| 537714    | 5/1987  | Canada         | . |
| 1277528   | 10/1970 | United Kingdom | . |
| 1515039   | 6/1976  | United Kingdom | . |
| 1573645   | 4/1977  | United Kingdom | . |
| 2 176 178 | 12/1986 | United Kingdom | . |

Primary Examiner—Edward A. Miller  
Attorney, Agent, or Firm—Pillsbury Madison & Sutro LLP

[57] 

### ABSTRACT

Compositions are provided which, when burned, produce significant levels of infrared radiation, but only limited levels of visible radiation. The basic components of the compositions include a binder, an oxidizer, and an organic fuel. Preferred oxidizers include those compounds which produce large quantities of infrared radiation when the flare composition is burned. Such oxidizers include potassium nitrate, cesium nitrate, rubidium nitrate, and combinations of these compounds. The composition preferably includes significant quantities of cesium nitrate as an oxidizer. Selection of the binder is important in order to provide the composition with the desirable characteristics identified above. The binder of the present invention does not produce significant soot when burned. At the same time, the binder serves to form a composition which is processible, avoids chunking, and is compatible with the oxidizers used. It has been found that polymer binders which include relatively short carbon chains (1–6 continuous carbon atoms) are preferred. Examples of such polymers include polyesters, polyethers, polyamides, and polyamines. Similarly, non-soot producing organic fuels are employed.

13 Claims, No Drawings

## 1

## PRESSABLE INFRARED ILLUMINANT COMPOSITIONS

This application is a continuation of U.S. application Ser. No. 07/913,841, filed Jul. 15, 1992, for PRESSABLE INFRARED ILLUMINANT COMPOSITIONS, and now abandoned.

### BACKGROUND

#### 1. The Field of the Invention

The present invention is related to illuminant compositions which emit significant quantities of infrared radiation. More particularly, the present invention is related to pressable/tampable infrared illuminant compositions which exhibit high initial burn rates, burn cleanly, and emit relatively small quantities of visible light in proportion to the infrared radiation emitted.

#### 2. Technical Background

There is a need in various situations for an ability to see clearly at night, or during periods of substantially reduced sunlight. Such situations may, for example, include search and rescue operations, police surveillance, and military operations. In these types of situations, it is often important that key personnel have the ability to see clearly, even though there is limited sunlight.

In order to solve the problem of visibility at night, or during periods of substantially reduced sunlight, devices have been developed which allow one to see based upon available infrared illumination, rather than visible light. While the infrared vision devices take on various configurations, perhaps the most common type of infrared vision devices are night vision goggles. These devices provide individual users with the ability to see much more clearly at night, while not significantly limiting the mobility of the individual user.

In order to facilitate the use of infrared vision devices, it has been found advantageous to enhance the available infrared radiation in the area of interest. In that regard, infrared emitting flare mechanisms have been developed. Such mechanisms have taken on a variety of configurations; however, the most widely used mechanisms comprise flares which emit relatively large quantities of infrared radiation in addition to any visible light that may be produced.

Infrared emitting flares are generally configured in much the same manner as visible light emitting flares. Such flares may provide infrared radiation at a single position on the ground, or they may provide such radiation above the ground. In the case of above-ground operation, the flare system includes an internal or external means of propulsion which allows the user to fire the flare in a desired direction. In addition, the flare itself includes a material which, when burned, produces significant quantities of infrared radiation. In general operation the flare is propelled over the area of interest and ignited. The emitted infrared radiation then greatly enhances the usefulness of infrared viewing devices, such as night vision goggles.

A number of problems have been encountered in the development of suitable infrared emitting compositions for use in such flares. For example, it will be appreciated that it is often desirable to provide an infrared emitting flare which does not emit excessive quantities of visible light. In situations where it is desirable to conduct operations under cover of night with a degree of secrecy, this capability is imperative. Excessive emission of visible light from the flare may alert individuals in the area to the existence of the flare,

## 2

which may in turn significantly reduce the effectiveness of the overall operation.

It has been found with known infrared flare compositions that excessive visible light is in fact emitted. In that regard, the performance of infrared emitting devices can be judged by the ratio of the amount of infrared radiation emitted to the amount of visible light emitted. This ratio is found to be low for many conventional infrared emitting compositions, indicating a high proportion of visible light being emitted from the flare.

Another problem encountered in the use of infrared emitting compositions relates to the burn rate achieved. Many known compositions have burn rates which are lower than would be desired, resulting in less infrared radiation than would be desired. In order to provide an effective flare, relatively high burn rates are required.

It is often observed that the burning (surface area) of the flare composition increases dramatically over time. This characteristic is also generally undesirable. In the case of an infrared emitting flare which is launched into the air, this means that less infrared radiation is emitted when the flare is high above the surface, while more infrared radiation is emitted while the flare is near the surface. Indeed, it is often found that the flare continues to burn after it has impacted with the ground.

It will be appreciated that this burn rate curve is just the opposite of that which would be generally desirable. It is desirable to have a high intensity infrared output when the flare is at its maximum altitude in order to provide good illumination of the ground. It is less critical to have high infrared output as the flare approaches the ground simply because the distance between the ground and the flare is not as great (illumination can be expressed by the equation  $\text{Illumination} = (I \times 4\pi) / (4\pi R^2)$  where  $I$  is the intensity in watts/steradian,  $R$  is the distance in feet from the flare to the object being illuminated, and illumination is expressed in units of watts/feet<sup>2</sup>). Ultimately, it is desirable that the flare cease operation before impact with the surface in order to reduce detection and obvious problems, such as fire, which may be caused when a burning flare impacts with the ground.

Another problem often encountered with known infrared emitting materials is "chunking out." This phenomenon relates to breakup or unbending separation of the flare illuminant grain during operation. In these situations it is found that large pieces of the infrared emitting composition may break away from the flare and fall to the ground. This is problematic because the flare fails to operate as designed when large pieces of the infrared producing composition are missing, the amount of infrared output over the subject location is curtailed, and falling pieces of burning flare material create a safety hazard.

It has also been found that the use of conventional flare compositions results in soot formation. Soot formation can adversely affect the operation of the flare device in several ways, including causing an increase in visible light emitted. When soot or carbon is heated it may radiate as a blackbody radiator. Soot formation is encountered primarily due to the fuels and binders employed in the infrared producing composition. Conventional infrared producing compositions have generally been unable to adequately deal with the problem of soot formation.

A further problem relates to aging of the IR emitting composition. It is often observed that known compositions substantially degrade over time. This is particularly true if the storage temperature is elevated. In some situations, it may be necessary to store these materials for long periods of

time at temperatures at or above 120° F. This has not been readily achievable with known compositions.

In summary, known infrared emitting compositions have been found to be less than ideal. Limitations with existing materials have curtailed their effectiveness. Some of the problem areas encountered have included low overall burn rates, undesirable burn rate curves, chunking out, poor aging, and undesirable levels of visible emissions.

It would, therefore, be a significant advancement in the art to provide infrared emitting compositions which overcame some of the serious limitations encountered with known compositions. It would be an advancement in the art to provide compositions which provided high levels of infrared emissions, while limiting the level of visible light output. It would be another significant advancement in the art to provide such compositions which had acceptably high burn rates.

It would also be an advancement in the art to provide infrared emitting compositions which substantially eliminated soot formation and which also substantially eliminated chunking. It would also be an advancement in the art to provide compositions which did not readily degrade with age, even when stored at relatively elevated temperatures.

Such compositions and methods are disclosed and claimed herein.

#### BRIEF SUMMARY AND OBJECTS OF THE INVENTION

The present invention is related to novel and inventive compositions which produce significant quantities of infrared radiation when burned. At the same time, the compositions avoid many of the limitations of the existing art. The compositions are pressable/tampable compositions, have high burn rates, produce relatively little visible light in proportion to infrared radiation produced (in that they substantially avoid soot formation). The compositions also avoid common problems such as chunking and poor high temperature aging.

The basic components of the compositions include a binder, an oxidizer, and a fuel. The fuels may preferably include nitrogen containing compounds. Other optional ingredients may also be added in order to tailor the characteristics of the composition to a specific use. Such optional ingredients include combustion rate catalysts and heat producing materials.

Preferred fuels fall into several related groups. One type of preferred fuel comprises molecules containing 3 to 6 member heterocyclic rings, and 1 to 4 nitrogen or oxygen atoms in the ring. Alkali metal salts of such heterocyclic compounds are also excellent fuels, as are bridged polycyclic amines. In addition, materials such as urea, guanidine, azodicarbonamide, and short chain alkyls fall within the scope of the present invention. All of these fuels result in very little soot production in the context of the present invention.

As mentioned above, it is critical to reduce visible light produced. This severely limits the fuels that can be used. Boron and silicon have been used in small amounts and act well as heat sources and as combustion rate catalysts. In addition, these materials are known to have some atomic emission lines located outside the visible spectrum, while producing tolerable amounts of visible light.

Hydrocarbon fuels have been evaluated and many tend to produce soot, which can lead to high visible light output. The hydrocarbon fuels/binders used, therefore, must burn

cleanly and provide nonluminous fragments that can burn with ambient air in the plume in order to increase the heat output and size of the radiation surface. At the same time, the material must serve to form a composition which is processible, avoids chunking, and is compatible with the oxidizers used.

The hydrocarbon binders (polymers) that have proven to reduce soot formation include polyesters, polyethers, polyamines, polyamides; particularly those with short carbon fragments in the backbone, alternating with oxygen or nitrogen atoms. It has been found that polymer binders which include relatively short carbon chains (about 1-6 continuous carbon atoms) are preferred. These molecules do not generally produce significant soot. Further, the additional desirable features of the invention can be achieved using these materials.

Preferred oxidizers include those compounds which produce large quantities of infrared radiation when the flare composition is burned. Such oxidizers include potassium nitrate, cesium nitrate, rubidium nitrate, and combinations of these compounds. These oxidizers are chosen to contain a metal with characteristic radiation wavelength in the near infrared (0.700 to 0.900 microns). The primary radiation comes from this line, whose width has been greatly broadened by the thermal energy in the plume.

It is believed to be important to provide free metal (potassium, cesium, or rubidium) during the burning of the flare composition in order to produce significant levels of infrared radiation. These metals appear to augment one another when used in certain combinations.

Significantly, high levels of cesium nitrate in the composition are found to greatly increase performance. Cesium nitrate is found to provide several significant advantages. Cesium nitrate is found to accelerate the burn rate. In addition, cesium nitrate broadens the infrared spectral output and improves infrared efficiency. Accordingly, it is preferred that cesium nitrate form from about 10% to about 90%, by weight, of the overall composition. In particular, excellent results are achieved when cesium nitrate is added to make up from about 25% to about 90% of the composition.

It is found that the compositions of the present invention produce relatively high burn rate materials. Burnrates at ambient pressures in the range of from about 0.0300 to about 0.1500 inches/second, and even somewhat higher, are readily achievable using the present invention. The more preferred range is above about 0.060 inches/second. Conventionally, it has been found that burn rates in this range are not readily achievable.

The present invention maintains the capability of tailoring desired characteristics by selecting specific combinations of fuels, oxidizers, and binders. Thus, particular burn rates and burn rate curves can be produced, the ratio of infrared radiation to visible light can be optimized, and the general physical and chemical properties can be carefully selected. Thus, the present invention provides a flexible illuminant material.

Accordingly, it is a primary object of the present invention to provide infrared emitting compositions which overcome several of the serious limitations encountered with known compositions.

It is an object of the present invention to provide compositions which when burned produce high levels of infrared emissions, while limiting the level of visible light output.

It is also an object of the present invention to provide such compositions which have high burn rates.

It is another object of the present invention to provide infrared emitting compositions which produce only limited soot and, therefore, limited visible output.

It is a further object of the invention to provide compositions which substantially eliminate chunking.

It is a further object of the present invention to provide compositions which do not significantly degrade with age, even when stored at relatively elevated temperatures.

These and other objects and advantages of the invention will become apparent upon reading the following detailed description and appended claims.

#### DETAILED DESCRIPTION OF THE PREFERRED EMBODIMENTS

As mentioned above, the present invention is related to pressable/tampable illuminant compositions which emit significant quantities of infrared radiation. The present invention also provides infrared propellant compositions which exhibit high initial burn rates, burn cleanly, and emit relatively small quantities of visible light in relation to the infrared radiation emitted.

As the title implies, pressable/tampable compositions are pressed into the desired configuration. This is a convenient form for illuminant to take and is readily usable in flares and related devices. Methods of pressing the illuminant compositions into the desire configurations are known in the art. One suitable method and apparatus for pressing infrared illuminant compositions is disclosed in U.S. Pat. No. 5,056,435 to Jones et al., which is incorporated herein by this reference. Other conventional foot presses may also be used because the compositions of the present invention exhibit significantly less chunking than conventional formulations, and are even significant improvements over the formulations disclosed in U.S. Pat. No. 5,056,435.

A typical pressable/tampable composition will include the following components in the following percentages by weight:

| Materials                                                              | Percent |
|------------------------------------------------------------------------|---------|
| Oxidizing Salt(s)<br>(such as Potassium Nitrate<br>and Cesium Nitrate) | 40-94   |
| Boron                                                                  | 0-10    |
| Silicon                                                                | 0-25    |
| Organic Fuel                                                           | 0-40    |
| Polymer Binder                                                         | 1-35    |

In most formulations, the percentage of organic fuel will be in the range of from about 5% to about 40%.

It will be appreciated that equivalent materials may be substituted for those identified above. Specifically, the nitrate salts may be substituted for one another, depending on the specific characteristics desired. One such example is rubidium nitrate, which may be added to the compositions, or may be substituted for some or all of the identified oxidizers. The ultimate objective in that regard is to provide a strong oxidizer which is also capable of substantially contributing to the output of infrared radiation during burning of the composition. The identified compounds possess those characteristics.

As mentioned above, the use of high levels of cesium salts (such as cesium nitrate) increases the burning rate by as much as 400% and reduces visible output by up to 50%. This occurs while at the same time maintaining high levels of infrared light in the 700 to 1100 nm region. Thus, specifically tailored formulations may include high levels of cesium nitrate in order to achieve specific performance criteria. It is presently preferred that the composition include

from about 10% to about 90% cesium nitrate. In some embodiments of the invention the preferred range will be from about 25% to about 80% cesium nitrate. It will be appreciated that the cesium nitrate comprises a portion of the total oxidizing salt added to the composition.

The compositions also include a polymer binder. The binder facilitates the formulation, processing, and use of the final composition. At the same time, the binder provides a source of fuel for the composition. Suitable binders in the present invention also insure a clean burning composition by substantially reducing soot formation.

As mentioned above, binders which are preferred in the present invention include polymers which have relatively short carbon chains (1-6 continuous carbon atoms) connected together by ether, amine, ester, or amide linkages (polyethers, polyamines, polyesters, or polyamides). Examples of such polymers include polyethylene glycol, polypropylene glycol, polybutylene oxide, polyesters, and polyamides. Binders of this type are commercially available and are well known to those skilled in the art.

A specific example of a suitable binder is Formrez 17-80 polyester of Witco Chemical Corp. and more particularly, a curable polyester resin composition comprising by weight, from about 81% to about 83% to, preferably about 82.5% Formrez 17-80 polyester resin, about 15 to about 17%, preferably about 16.5% epoxy such as ERL 510 of Ciba-Geigy Corporation and about 0 to about 2%, and preferably 1% of a catalyst such as iron linoleate. More preferably, the binder may comprise about 82.5% Formrez 17-80 polyester resin, about 16.5% ERL epoxy and about 1% iron linoleate. Such a binder composition is referred to herein as WITCO 1780.

As discussed above, in the pressable/tampable compositions of the present invention, a separate fuel is provided. Fuels which fall within the scope of the present invention include nitrogen and oxygen containing compounds. One type of fuel comprises molecules with 3 to 6 member heterocyclic rings, which also contain 1 to 4 nitrogen and/or oxygen atoms in the ring. Examples of such compounds include tetrazoles, triazoles, triazines, imidazoles, oxazole, pyrazole, pyrrolidine, pyrrolinidine, pyridine, pyrimidine, and similar compounds.

Combinations of such ring systems can be fused or joined by covalent bonds, such as in bitetrazole. Such heterocyclic rings may be substituted with nitrogen containing groups (such as nitro, nitroso, cyano, and amino) at any or all substitutable sites on the ring. Alkali metal salts of such heterocyclic compounds, or their derivatives, are also useful. Preferred alkali metal include potassium, rubidium, and cesium, alone or in combination.

Bridged polycyclic amines are also useful as fuels. Also useful are salts arising from combinations of polycyclic amines and organic or inorganic acids. Such compounds include dicyanidamide, cyanonitramide, hydrogencyanide, dicyanamide, and the like.

Other related materials are also found to serve well as fuels in the present invention. Such materials include urea, guanidine, azodicarbonamide, and short chain alkyls that contain 1 to 8 carbons. In addition, derivatives of such compounds, substituted with nitrogen containing groups, are also useful. Substitution may be made with  $\text{NO}_2$ ,  $\text{NO}$ ,  $\text{CN}$ , and/or  $\text{NH}_2$ .

It is apparent that the fuels must burn cleanly, rapidly, and at high temperatures. The fuels do not produce significant amounts of soot, with its associated increase in visible light output. The fuels identified above meet these performance criteria.

As mentioned above, it is also possible to add combustion rate catalysts and heat sources to the overall composition. These materials provide for further tailoring of the performance characteristics of the resulting composition. These materials, however, must also fit the other parameters of an acceptable composition such as producing little visible light and not contributing to the other undesirable characteristics identified herein. Two examples of such preferred materials include silicon and boron, while magnesium is not preferred because of its propensity to emit large quantities of visible light.

In the pressable/tampable compositions described herein, boron is preferably added to constitute from about 0% to about 10%, by weight of the total composition. Silicon preferably makes up from about 0% to about 25% of the total composition.

One measure of a preferred composition is the ratio of infrared radiation to visible light produced during burning of the composition. Preferably the composition will have an IR/Vis. ratio of at least 3.50, and more preferably greater than 6.0. Indeed, ratios of from about 10 to about 20 are achievable with the present invention. These levels of infrared output per unit of visible output have not been easily achievable using conventional compositions.

It is found that the compositions within the scope of the present invention also provide increased burn rates. Burn rates within the range of about 0.030 to about 0.150 inches per second, and even above, are characteristic of the compositions of the present invention. As mentioned above, the preferred burn rates are in excess of 0.060 inches/second.

Compositions within the scope of the present invention also age and store well. It has been found that a composition was still acceptable after being stored at 135° F. for one year. This is a further feature which has not generally been available in known compositions.

Compositions within the scope of the present invention can be formulated and prepared using known and conventional technology. Formulation techniques such as those generally employed in mixing and preparing propellant, explosive, and pyrotechnic compositions are preferably used in the preparation of the compositions within the scope of the present invention.

### EXAMPLES

The following examples are given to illustrate various embodiments which have been made or may be made in accordance with the present invention. These examples are given by way of example only, and it is to be understood that the following examples are not comprehensive or exhaustive of the many types of embodiments of the present invention which can be prepared in accordance with the present invention.

#### Example 1

In this example a composition within the scope of the present invention was formulated and tested. A mixture of the ingredients listed below was made and pressed into pellets weighing approximately 3 grams.

| Material                   | Percentage (by weight) |
|----------------------------|------------------------|
| KNO <sub>3</sub>           | 70.0                   |
| Potassium dicyanoimidazole | 15.0                   |
| Silicon                    | 7.0                    |
| Boron                      | 2.0                    |
| Witco Binder Premix        | 6.0                    |

The Witco Binder Premix comprised a mixture of WITCO 1780 liquid polyester (triethyleneglycol succinate), manu-

factured by Witco Corp, blended with an appropriate amount of an epoxy curing agent to provide adequate cure.

The pellet was then burned and the burn rate, output of visible light and output of infrared radiation were measured. Visible light was measured with a silicon photodiode with photopic response. Infrared radiation was measured using a silicon cell with a 695 nm cut on filter. Tests on the composition yielded the following data:

|    |           |                   |
|----|-----------|-------------------|
| 10 | WEB       | 0.500 inches      |
|    | Weight    | 3.008 grams       |
|    | Burntime  | 8.57 seconds      |
| 15 | Burnrate  | 0.057 inches/sec. |
|    | Avg. IR   | 701.57 mV         |
|    | Avg. Vis. | 94.02 mV          |
|    | IR/Vis.   | 7.47              |

All data represent the average of three runs.

As can be seen from the data presented above, the composition provides a useful infrared emitting composition. The composition provides a rapid burn rate, along with high IR output and relatively low visible output.

#### Example 2

In this example a composition within the scope of the present invention was formulated and tested. A mixture of the ingredients listed below was made and pressed into pellets weighing approximately 3 grams.

| Material             | Percentage (by weight) |
|----------------------|------------------------|
| KNO <sub>3</sub>     | 70.0                   |
| 4,5-dicyanoimidazole | 15.0                   |
| Silicon              | 7.0                    |
| Boron                | 2.0                    |
| Witco Binder Premix  | 6.0                    |

The pellet was then burned and the burn rate, output of visible light, and output of infrared radiation measured. Tests on the composition yielded the following data:

|    |           |                   |
|----|-----------|-------------------|
| 50 | WEB       | 0.521 inches      |
|    | Weight    | 3.071 grams       |
|    | Burntime  | 13.13 seconds     |
|    | Burnrate  | 0.040 inches/sec. |
|    | Avg. IR   | 560.20 mV         |
|    | Avg. Vis. | 73.03 mV          |
|    | IR/Vis.   | 7.67              |

All data represent the average of three runs.

As can be seen from the data presented above, the composition provides a useful infrared emitting composition. The composition provides a rapid burn rate, along with high IR output and relatively low visible output.

#### Example 3

In this example a composition within the scope of the present invention was formulated and tested. A mixture of the ingredients listed below was made and then burned.

| Material            | Percentage (by weight) |
|---------------------|------------------------|
| KNO <sub>3</sub>    | 64.0                   |
| Dicyanoimidazole    | 15.0                   |
| Silicon             | 15.0                   |
| Witco Binder Premix | 6.0                    |

The burn rate, output of visible light, and output of infrared radiation measured. Tests on the composition yielded the following data:

|           |                |
|-----------|----------------|
| WEB       | 0.499 inches   |
| Burnrate  | 0.0391 in/sec. |
| Burntime  | 12.76 seconds  |
| Avg. IR   | 467.03 mV      |
| Avg. Vis. | 64.00 mV       |
| IR/Vis.   | 7.28           |

All data represent the average of three runs.

As can be seen from the data presented above, the composition provides a useful infrared emitting composition. The composition provides a rapid burn rate, along with high IR output and relatively low visible output.

#### Example 4

In this Example a composition within the scope of the present invention was formulated and tested. The following ingredients were mixed to produce an infrared emitting composition:

| Material          | Percentage (by weight) |
|-------------------|------------------------|
| KNO <sub>3</sub>  | 50.0                   |
| CsNO <sub>3</sub> | 10.0                   |
| Si                | 14.0                   |
| B                 | 4.0                    |
| Witco             | 6.0                    |
| Melamine          | 16.0                   |

The composition was aged for 6 months at 135° F. The composition was then burned in a flare of 2.75 inches diameter, 13.1 inches in length, and weighing 5 pounds. The following results were obtained and are the average for four separate tests:

|           |                      |
|-----------|----------------------|
| Burntime  | 159.6 seconds        |
| Burnrate  | 0.0773 inches/second |
| Avg. IR   | 2.352 V              |
| Avg. Vis. | 346.1 mV             |
| Area IR   | 374.7 V sec.         |
| Area Vis. | 55.15 V sec.         |
| IR/Vis.   | 6.79                 |

A high output of infrared was achieved early in the burn sequence and was then sustained. At the same time, the IR to visible ratio was well within acceptable ranges.

It can be appreciated from the results achieved that an acceptable infrared emitting composition was produced. Furthermore, the results clearly indicate that the composition remained usable even after storage at elevated temperature for 6 months.

#### Example 5

In this Example a composition within the scope of the present invention is formulated. The following ingredients are mixed to produce an infrared emitting composition:

| Material          | Percentage (by weight) |
|-------------------|------------------------|
| CsNO <sub>3</sub> | 80.0                   |
| Si                | 20.0                   |
| Witco             | 6.0                    |

This material provides an infrared producing composition within the scope of the present invention. Expected data from such a formulation would be as follows:

|           |                     |
|-----------|---------------------|
| Burntime  | 4.5 seconds         |
| Burnrate  | 0.080 inches/second |
| Avg. IR   | 2.60 V              |
| Avg. Vis. | 260 mV              |
| IR/Vis.   | 10.0                |

20

#### Example 6

In this Example a composition within the scope of the present invention is formulated. The following ingredients are mixed to produce an infrared emitting composition:

| Material             | Percentage (by weight) |
|----------------------|------------------------|
| CsNO <sub>3</sub>    | 45.0                   |
| KNO <sub>3</sub>     | 35.0                   |
| Si                   | 10.0                   |
| Boron                | 4.0                    |
| polypropylene glycol | 6.0                    |

30

This material provides an infrared producing composition within the scope of the present invention.

#### Example 7

In this example, a composition within the scope of the present invention was tested in terms of aging, and compared to a hexamine-containing control formulation. Standard temperature and humidity aging tests were preformed.

The composition within the scope of the present invention contained Witco binder, melamine, and KNO<sub>3</sub>. The control composition contained Witco binder, hexamine, and KNO<sub>3</sub>. The compositions were formed into standard flares and were aged pursuant to military standard MIL-STD-331B, temperature and humidity cycle single chamber method. The flares were conditioned for two consecutive 14-day cycles, for a total of 28 days. Flight and tower tests were performed. It was observed that the control developed cracking at several locations, while the composition within the scope of the invention exhibited no apparent physical change or performance degradation.

55 Three flares of each type were tested, and visible energy, infrared energy, and burn rate data were collected.

After the first 14-day cycle, one flare from each formulation was dissected. Two flares were burned. The most notable change was an increase in chunking by the control.

50 After the full 28-day cycle, one flare from each formulation was dissected. The control was found to have four grain cracks, while the formulation tested had none.

Two flares were burned to measure performance. Data for the baseline, 14-day, and 28-day cycle tests are as shown below:

65

|                 | Control      |              |              |    |
|-----------------|--------------|--------------|--------------|----|
|                 | Baseline     | 14-Day Cycle | 28-Day Cycle |    |
| Average IR      | 2.15 V       | 2.19 V       | 2.293 V      | 5  |
| Average Vis.    | 315 mV       | 303 mV       | 304 mV       |    |
| IR/Vis.         | 6.8          | 7.2          | 7.5          |    |
| Burnrate        | 0.043 in/sec | 0.041 in/sec | 0.042 in/sec |    |
| Burntime-tower  | 320 sec      | 311 sec      | 317 sec      |    |
| burntime-flight | 201 sec      | —            | —            | 10 |
| grain cracks    | 0            | 3            | 4            |    |
| flight chunks   | 1            | —            | —            |    |
| tower chunks    | 0            | 1            | 2            |    |

  

|                 | Test Composition |              |              |    |
|-----------------|------------------|--------------|--------------|----|
|                 | Baseline         | 14-Day Cycle | 28-Day Cycle |    |
| Average IR      | 1.59 V           | 1.74 V       | 1.82 V       |    |
| Average Vis.    | 263 mV           | 299 mV       | 290 mV       |    |
| IR/Vis.         | 6.1              | 5.8          | 6.3          |    |
| Burnrate        | 0.068 in/sec     | 0.073 in/sec | 0.070 in/sec |    |
| Burntime-tower  | 185 sec          | 170 sec      | 180 sec      |    |
| Burntime-flight | 205 sec          | —            | —            | 25 |
| grain cracks    | 0                | 0            | 0            |    |
| flight chunks   | 0                | —            | —            |    |
| tower chunks    | 0                | 0            | 0            |    |

Accordingly, it can be seen that compositions within the scope of the present invention provide significantly improved aging characteristics. No chunking or cracking was observed using the invention composition. Using the hexamine-containing control, however, cracking and chunking were observed over the course of the tests.

## SUMMARY

In summary, the present invention provides new and useful illuminant formulations which produce large quantities of infrared radiation, but produce relatively small quantities of visible light. Accordingly, some of the major drawbacks with known infrared producing materials are avoided.

The compositions of the present invention have high burn rates. The compositions emit infrared while producing only limited soot and, therefore, limited visible light is produced. The compositions of the present invention also substantially eliminate chunking. The compositions do not significantly degrade with age, even when stored at relatively elevated temperatures. Thus, the compositions of the present invention represent a significant advancement in the art.

The invention may be embodied in other specific forms without departing from its spirit or essential characteristics. The described embodiments are to be considered in all respects only as illustrative and not restrictive. The scope of the invention is, therefore, indicated by the appended claims rather than by the foregoing description. All changes which come within the meaning and range of equivalency of the claims are to be embraced within their scope.

What is claimed and desired to be secured by United States Letters Patent is:

1. An infrared producing illuminant composition which consists essentially of:

from about 40% to about 90% by weight alkali metal oxidizer salt, wherein said alkali metal oxidizer salt is selected from the group consisting of potassium, cesium, and rubidium oxidizer salts, and mixtures thereof, wherein the amount of potassium oxidizer salt is limited such that the infrared producing illuminant composition has at least 25% by weight cesium oxidizer salt;

a combustion rate catalyst which is at least one of boron or silicon, wherein the boron is in an amount of from about 0% to about 10%, and wherein silicon is present in an amount of from about 0% to about 25%; from about 1% to about 35% by weight polymer binder which is not hexamine,

wherein upon burning, the infrared illuminant composition produces little or no visible light such that the ratio of infrared radiation to visible radiation is greater than approximately 6.0, and wherein the infrared producing illuminant composition has a burn rate greater than 0.060 inches/second.

2. An infrared producing illuminant composition as defined in claim 1, wherein said combustion rate catalyst contains (i) 15.0% by weight silicon, (ii) 2.0% by weight of boron, (iii) 14.0% by weight silicon and 4.0% by weight boron, (iv) 20.0% by weight silicon, or (v) 10.0% by weight silicon and 4.0% by weight boron.

3. An infrared producing illuminant composition consisting essentially of:

from about 40% to about 90% by weight alkali metal oxidizer, wherein said alkali metal oxidizer is selected from the group consisting of potassium, cesium, and rubidium oxidizer salts, and mixtures thereof, wherein the amount of potassium oxidizer salt is limited such that the infrared producing illuminant composition has at least 25% by weight cesium oxidizer salt;

from about 1% to about 35% by weight binder; and from about 5% to about 40% by weight organic fuel, distinct from the binder, wherein said organic fuel is selected from the group consisting of tetrazoles, triazoles, triazines, imidazoles, oxazole, pyrazole, pyrrolidine, pyrrolinidine, pyridine, pyrimidine, derivatives thereof substituted with substituent group(s) selected from the group consisting of  $-\text{NO}_2$ ,  $-\text{NO}$ ,  $-\text{CN}$ , and  $-\text{NH}_2$ , alkali metal salts thereof, melamine, and mixtures thereof,

wherein upon burning, the infrared producing illuminant composition produces little or no visible light such that the ratio of infrared radiation to visible radiation is greater than approximately 6.0, and wherein the infrared producing illuminant composition has a burn rate greater than 0.040 inches/second.

4. An infrared producing illuminant composition formulated from ingredients which consist essentially of:

from about 40% to about 90% by weight alkali metal oxidizer salt, wherein said alkali metal oxidizer salt is selected from the group consisting of potassium, cesium, and rubidium oxidizer salts, and mixtures thereof, said composition having at least about 25% by weight cesium nitrate;

from about 1% to about 35% by weight binder which is at least one selected from the group consisting of polyethylene glycol, polypropylene glycol, polybutylene oxide, polyester, and polyamide;

at least one combustion rate catalyst which is at least one of boron or silicon, wherein the boron is present in an amount of from about 0% to about 10%, and, silicon is present in an amount of from about 0% to about 25%; from about 5% to about 40% by weight organic fuel which is selected from the group consisting of tetrazoles, triazoles, imidazoles, oxazole, melamine, pyrazole, pyrrolidine, pyrrolinidine, pyridine, and pyrimidine;

wherein, upon burning, the composition produces little or no visible light such that the ratio of infrared radiation

**13**

to visible radiation is greater than approximately 3.5, and wherein the infrared producing illuminant composition has a burn rate greater than 0.060 inches/second.

**5.** An infrared producing illuminant composition according to claim **3** or **4**, wherein said alkali metal oxidizer salt is a combination of potassium nitrate and cesium nitrate. <sup>5</sup>

**6.** An infrared producing illuminant composition according to claim **3** or **4**, wherein said infrared producing illuminant composition contains from about 25% to about 80% by weight of cesium nitrate.

**7.** An infrared producing illuminant composition according to claim **4**, wherein said combustion rate catalyst is a combination of silicon and boron.

**8.** An infrared illuminant composition according to claim **3** or **4**, wherein said organic fuel is melamine.

**9.** An infrared producing illuminant composition according to claim **3**, wherein said infrared producing illuminant composition consists essentially of

45% by weight of cesium nitrate, 35% by weight of potassium nitrate, 10% by weight of silicon, 4% by weight of boron, and 6% by weight of a binder mix which is based on polypropylene glycol.

**10.** An infrared producing illuminant composition pelletized from ingredients which consist essentially of:

from about 40% to about 90% by weight alkali metal oxidizer salt, wherein said alkali metal oxidizer salt is selected from the group consisting of potassium, cesium, and rubidium oxidizer salts, and mixtures thereof, wherein the infrared producing illuminant composition has at least 25% by weight cesium oxidizer salt; <sup>25</sup>

**14**

a combustion rate catalyst which is a combination of boron and silicon, wherein the boron is in an amount greater than about 0% and up to about 10%, and wherein silicon is present in an amount of greater than about 0% and up to about 25%;

from about 1% to about 35% by weight of at least one polymeric binder selected from the group, consisting of polyester, polyether, polyamine, and polyamide:

from about 1% to about 40% by weight of organic fuel which is not hexamine, whereby upon burning, the infrared illuminant composition produces little or no visible light such that the ratio of infrared to visible radiation is greater than approximately 3.5, and wherein the infrared producing illuminant composition has a burn rate greater than 0.060 inches/second.

**11.** An infrared producing illuminant composition according to claim **3**, wherein said binder is at least one polymer carbon chains of 1-6 continuous carbon atoms linked by ether, amine, ester or amide linkages.

**12.** A pressible infrared producing illuminant composition according to claim **10**, wherein said IR/visible light ratio is 10 to 20.

**13.** A pressible infrared producing illuminant composition according to claim **1**, wherein said binder is a curable polyester and an epoxy curing agent therefor.

\* \* \* \* \*